

1

2,781,318

## MINERAL LUBRICATING OIL ADDITIVE

Elmer B. Cyphers, Cranford, N. J., assignor to Esso Research and Engineering Company, a corporation of Delaware

No Drawing. Application March 28, 1952,  
Serial No. 279,205

5 Claims. (Cl. 252—47)

The present invention relates to the use of dialkyl phenothiazines as oil soluble ashless detergent additives for mineral lubricating oils.

In accordance with the present invention, the higher alkyl derivatives of phenothiazine have been found to be excellent additives for mineral lubricants employed in internal combustion engines. These additives are useful in maintaining cleanliness of engines operating under severe conditions, i. e., in minimizing formation of coke-like deposits, varnish and the like on various engine parts.

Phenothiazine has been suggested as antioxidant and corrosion inhibiting additive for ester, polyester, polyether, and other synthetic lubricants. However, in contrast to the effect of alkyl phenothiazines in mineral lubricants, the presence of phenothiazine in synthetic crankcase lubricants actually promotes deposit formation in internal combustion engines operating under severe conditions. This effect has greatly detracted from its utility. Phenothiazine has also been suggested as a corrosion inhibitor for mineral lubricants, very small concentrations being used for this purpose. However, phenothiazine does not aid in maintaining engine cleanliness when used in such compositions.

In view of the above matters, it was quite surprising to find that the higher alkyl phenothiazines are quite effective detergent additives for mineral motor oils and yet show substantially no corrosion inhibition properties. They are particularly useful as ashless detergents since they leave no deposits in the combustion chamber. This is a valuable property in the case of aviation lubricants where the presence of ash may lead to complete destruction of a piston in a matter of minutes due to preignition.

Moreover, phenothiazine and its lower alkyl derivatives are insoluble in mineral base lubricants in substantial concentrations and the usual solubilizers have failed to increase their solubility to a useful level. However the higher alkyl phenothiazine derivatives of the present invention are soluble in effective concentrations in mineral lubricants over a wide range of temperatures that would normally be encountered in storage, transportation and use.

The reason for the different effects obtained when using phenothiazine and higher alkyl phenothiazines in mineral and synthetic lubricants is not understood. While it is not desired to be limited as to any theory of action, obviously such compounds act by entirely different mechanisms. For example, in the case of synthetic and mineral lubricants, phenothiazine in small concentrations may inhibit formation of acids, hydroperoxides and other corrosive substances that might otherwise form through oxidation but exhibits no detergency characteristics. On the other hand, the compounds of this invention evidently have little effect on the formation of corrosive materials but they undoubtedly retard formation of condensation and polymerization products that lead to varnish and coke-like engine deposits. They may also help maintain engine cleanliness by keeping such oil insoluble materials in suspension in the oil.

2

The compounds of the present invention have the following general formula:



10 wherein the R groups are alkyl radicals, each having in the range of 4 to 16 carbon atoms, preferably 6 to 12 carbon atoms. The R groups may be similar or dissimilar but those that are identical in structure are preferred from the standpoint of ease of preparation. They are generally located in the para positions with respect to the nitrogen group, because of their relative ease of preparation. The R groups may be straight chain or branched in structure; branched groups are usually preferable from the standpoint of improving oil solubility. Specific alkyl groups include butyl, isopentyl, n-hexyl, tert.-octyl, n-decyl, dodecyl and the like.

15 The dialkyl phenothiazines are readily prepared by analogous procedures used for making phenothiazine. For example, a dialkyl diphenyl amine may be treated with sulfur at an elevated temperature, such as one in the range of about 300°—400° F. for a sufficient time to complete the reaction. The reaction may be carried out in the presence of a catalyst such as iodine. The reaction products may be purified by washing with suitable solvents, crystallization, recrystallization and the like procedures.

20 The dialkyl phenothiazine may be blended in mineral lubricating oils in amounts in the range of about 0.2 to 5% by weight, the upper limit being restricted to some extent by the solubility of the particular compound being used. Thus, the dibutyl derivatives will generally be soluble to the extent of only about 1.0% whereas the higher alkyl derivatives are soluble to a greater extent. A preferred concentration is in the range of about 0.5 to 1.5% by weight.

25 The additives of the present invention are particularly suitable for aviation engine lubricants, although they will find use as additives for other types of combustion engine lubricants, diesel lubricants, etc. The lubricating oil base stocks may be derived from petroleum distillates and residuals refined by conventional means. Other agents may be employed in the oil compositions. Such agents include pour point depressants, viscosity index improvers, oiliness agents and the like.

30 The invention will be more fully understood by reference to the following examples. These examples, however, are given for the purpose of illustration only and are not to be construed as limiting the scope of the present invention in any way.

### Example 1.—Preparation of dioctyl phenothiazine

35 470 g. (1.2 mols) of p,p'-diisooctyl diphenyl amine, 76.8 g. (2.4 mols) of sulfur and 4 g. iodine (employed as a catalyst) were mixed in a three-neck flask and were heated at a temperature of 340°—360° F. for 1.5 hours. The mixture was then cooled, diluted with three volumes of hexanes at 210° F., heated to boiling, and filtered while hot thru "Hi-flo" diatomaceous filter aid. The filtrate was then cooled to form crystals which were separated by filtration. The crystals were then dissolved in fresh hexane, a small amount of carbon black was added, and the mixture cooled to crystallize the product. The crystals were then recovered by filtration and washed with additional hexane. The product, p,p'-diisooctyl phenothiazine was a white, crystalline material having a melting point of 167° to 168° C., and nitrogen and sulfur contents of 3.11 weight percent and 7.36 weight percent, respectively.

*Example II.—Mineral oil solubility tests*

The solubility of phenothiazine and of the diethyl phenothiazine of Example I in mineral lubricating oils was determined in a series of tests. The tests were carried out employing as a lubricant base stock a Mid-Continent, solvent extracted aviation lubricating oil having a viscosity (Saybolt) at 210° F. of about 100 seconds.

The solubility of phenothiazine was determined by blending a desired amount of it in the base oil at a temperature of about 150° F., at which temperature the material was soluble, cooling the mixture down to 40° F., and observing the resulting oil blend. A blend containing 0.1% by weight phenothiazine remained clear for six months whereas blends containing in the range of 0.2 to 0.5 weight percent of this compound became cloudy within three to nine days.

Oil blends were prepared containing 0.5% phenothiazine and 0.5% of various solubilizers including "Lorol B" alcohol (C<sub>10</sub>-C<sub>18</sub> alcohols), diisooctyl adipate, dibutyl phthalate and diethyl phthalate. In each case, the oil blends contained sediment or were hazy or cloudy within from two to ten days at 40° F.

The diethyl phenothiazine of Example I was tested for solubility characteristics as above. An oil blend containing 1% by weight of this material remained clear for 30 days at a temperature of 40° F., after which the test was discontinued. This same blend remained clear for 2 months at both room temperature and 120° F., after which the tests were discontinued. A blend containing 1.5% of this compound was clear after 60 days at room temperature. A blend containing 2% of the product showed slight sediment in 7 days at room temperature.

*Example III.—Aviation C. F. R. engine evaluation*

A portion of the diethyl phenothiazine of Example I was evaluated as an additive in a solvent extracted Mid-Continent aviation oil base stock having a viscosity of 210° F. of about 100 Saybolt seconds. In one experiment, the base stock per se was tested, and in another the base stock containing 1% of diethyl phenothiazine was tested. The test consisted of operating the aviation C. F. R. engine for 25 hours at 1800 R. P. M. and 4 brake horsepower. The oils were rated on a demerit system wherein a perfectly clean surface is given a rating of 0 and a rating of 10 is given to the worst condition that could be expected. The results are shown in the following table.

| Additive in oil base stock             | Over-all | Ring zone | Varnish | Piston under-head | Ring sticking | Pin relief |
|----------------------------------------|----------|-----------|---------|-------------------|---------------|------------|
| None                                   | 2.6      | 6.0       | 3.3     | 4.0               | 3.1           | 4.6        |
| Diethyl phenothiazine, 1.0 wt. percent | 1.6      | 2.9       | 2.4     | 1.0               | 2.5           | 3.8        |

In the case of the base oil, the deposits in the critical ring zone area were quite heavy (6.0 demerit) and the addition of only 1% of diethyl phenothiazine resulted in a marked improvement (2.9 demerit). Appreciable improvement was also obtained in the piston underhead demerit by the use of the additive. It is seen that the dialkyl phenothiazines of the present invention are quite effective in helping maintain engine cleanliness in general and in imparting detergency characteristics to the oil.

*Example IV.—Lauson engine test on synthetic lubricant*

Phenothiazine was tested as an additive for a synthetic lubricant. The synthetic lubricant base stock employed was a C<sub>8</sub> "Oxo" adipate prepared by esterifying adipic acid with C<sub>8</sub> "Oxo" alcohol (from catalytic oxonation of C<sub>7</sub> olefins with hydrogen and carbon monoxide) to form the diester derivative. A portion of the base oil per se and of the base oil containing 0.5% by weight of phenothiazine were tested in a standard Lauson engine test which was conducted by operating the engine at 1800

R. P. M. for 25 hours with a 1.5 indicated kilowatt load, 300° F. oil temperature and 295° F. water jacket temperature. The oils were rated by the demerit system described in connection with the C. F. R. test (Example III). The loss in weight of the copper-lead bearings was also determined. The results are shown in the following table.

| 10  | Phenothiazine in C <sub>8</sub> "Oxo" adipate, wt. percent | Piston skirt varnish demerit | Cu-Pb bearing weight loss (g./bearing) |
|-----|------------------------------------------------------------|------------------------------|----------------------------------------|
| 0.  |                                                            | 0.3                          | ( <sup>1</sup> )                       |
| 0.5 |                                                            | 6.5                          | 0.39                                   |

<sup>1</sup> Bearing failure at 22.5 hours.

The presence of only 0.5 weight percent of phenothiazine in the synthetic lubricant promoted engine deposit formation, the blend being much worse in this respect than the base oil. This is in marked contrast to the improved detergency characteristics obtained by using the dialkyl phenothiazine in a mineral lubricant as shown in Example III. The phenothiazine however demonstrated potent corrosion inhibition properties and prevented bearing failure.

*Example V.—Chevrolet engine tests*

An S. A. E. grade mineral lubricant base oil (derived from acid-treated Mid-Continent lubricant stocks) was tested, with and without various additives, in a Chevrolet engine. The test, known as the Chevrolet L4 Test, was carried out for 36 hours. In one test the base oil contained 5% of a conventional detergent additive (termed herein Detergent Additive A) comprising calcium petroleum sulfonate and metal alkyl phenol sulfides. In another test, the oil contained 5% of Detergent Additive A and 0.5% by weight of phenothiazine. In another test, the oil contained 5% of Detergent Additive A and 0.5% by weight of the diethyl phenothiazine of Example I. Varnish demerit ratings and loss in weight of copper-lead bearings were determined for each run as follows:

| 45                                          | Additive in base oil | Piston skirt varnish demerit | Cu-Pb bearing weight loss, g./bearing |
|---------------------------------------------|----------------------|------------------------------|---------------------------------------|
| None                                        |                      | 9.5                          | 0.71                                  |
| Additive A, 5%                              |                      | 2.2                          | 0.39                                  |
| Additive A, 5%; phenothiazine, 0.5%         |                      | 2.2                          | 0.09                                  |
| Additive A, 5%; diethyl phenothiazine, 0.5% |                      | 1.1                          | 0.37                                  |

Phenothiazine demonstrated corrosion inhibition properties but did not improve the detergency characteristics of the oil. The dialkyl phenothiazine, on the other hand, showed substantial detergent properties but no corrosion inhibition properties.

*Example VI.—Aluminum cup coking test*

An oil blend containing 0.5% of the diethyl phenothiazine of Example I in the aviation base oil described in Example III was evaluated in the aluminum cup coking test. This test determines the effectiveness of the additive as an inhibitor of coking under the severe temperature conditions generally encountered in aviation engines. The coking test was carried out by placing a desired amount of the base stock in an aluminum measuring cup and stirring while heat was applied. The side walls of the cup were maintained at a temperature of about 500° F. while the oil was heated from the bottom until it reached a temperature of 550° F. The stirrer was then stopped for 10 minutes, followed by stirring for 10 minutes. The alternate non-stirring and stirring periods were repeated until the end of the 4th non-stirring period. The oil was then discarded and the coke deposit weighed. A portion of the lubricant base oil containing no addi-

tive was also evaluated for comparative purposes. The results of the tests follow:

| Dioctyl phenothiazine in aviation base oil, weight percent | Aluminum cup test deposits, mg. coke per 75 g. of oil |
|------------------------------------------------------------|-------------------------------------------------------|
| None.....                                                  | 21                                                    |
| 0.5.....                                                   | 5                                                     |

The dialkyl phenothiazine is a potent inhibitor for minimizing coking of mineral lubricating oils.

The lubricating oil base stocks used in the compositions of this invention may be straight mineral lubricating oils or distillates derived from paraffinic, naphthenic, asphaltic or mixed base crudes, or, if desired, various blended oils may be employed as well as residuals, particularly those from which asphaltic constituents have been carefully removed. The lubricating oil base stocks will usually range from about 40 to 150 seconds (Saybolt) viscosity at 210° F. The viscosity index may range from 0 to 100 or even higher, although for aviation lubricants, which are the preferred base stocks in the practice of the present invention, the higher viscosity indexes are preferred.

What is claimed is:

1. A lubricant composition consisting essentially of a mineral oil and in the range of about 0.2 to 5.0% by

5 weight of a compound having the following general formula:



10 wherein the R groups are alkyl radicals, each having in the range of 4 to 16 carbon atoms.

15 2. A composition as in claim 1 in which said R groups are identical and have in the range of 6 to 12 carbon atoms.

3. A composition as in claim 2 wherein said R groups each contain 8 carbon atoms.

4. A composition as in claim 1 wherein said R groups are in the para positions.

15 5. A lubricating oil composition consisting essentially of a mineral lubricant base and in the range of 0.2 to 1.5% by weight of p,p'-diisooctyl phenothiazine.

References Cited in the file of this patent

UNITED STATES PATENTS

|           |                 |               |
|-----------|-----------------|---------------|
| 2,006,756 | Bartram         | July 2, 1935  |
| 2,190,648 | Cantrrell       | Feb. 20, 1940 |
| 2,587,660 | Smith           | Mar. 4, 1952  |
| 2,609,343 | Saunders et al. | Sept. 2, 1952 |